

## UNITED STATES PATENT OFFICE

2,041,728

## TEXTILE PROCESS

George Schneider, Montclair, N. J., assignor to  
Celanese Corporation of America, a corpora-  
tion of Delaware

No Drawing. Application September 14, 1933,  
Serial No. 689,403

21 Claims.

(Cl. 28—1)

This invention relates to a process of improving the properties of textile materials by incorporating in or applying thereto a polymerized oil or the like.

5 An object of the invention is the production of a yarn or the like which knits or weaves uniformly.

Another object is the formation of a yarn or fabric which readily and evenly takes a dye and one which delusters easily. Other objects will 10 be apparent from the following description.

15 My invention is applicable to artificial yarns and the like of organic derivatives of cellulose by applying to the same the polymerized oil with a softener or swelling agent to incorporate it therein, by applying the polymerized oil to the surface of the yarn as a coating, or by adding it to the solution from which artificial films or filaments are made.

20 My invention is applicable to the treatment of yarns or filaments, under which terms are included threads, assemblies or bundles of a number of continuous filaments which may be in parallel relationship or which may be twisted together, artificial bristles, straws, short lengths 25 of staple fibres, and yarn spun from such staple fibres.

30 This invention is particularly of importance in connection with the production of yarns or filaments made of organic esters of cellulose and cellulose ethers. Examples of cellulose esters are cellulose acetate, cellulose formate, cellulose propionate and cellulose butyrate, while examples of cellulose ethers are ethyl cellulose, methyl cellulose and benzyl cellulose. The invention is 35 also applicable to yarns or filaments made of reconstituted cellulose.

35 The polymerized oil may be applied to yarns or added to the spinning solution for forming synthetic yarns, which yarn or spinning solution may have therein effect materials such as pigments, filling materials, dyes or lakes; fire retardants such as beta chloronaphthalene, triphenyl phosphate or tricresyl phosphate. The 40 effect materials and fire retardants may also be applied as coatings before or after the application of my invention.

45 By utilization of my invention in connection with synthetic yarn, there is produced a yarn having substantially normal tenacity and elongation and which dyes darker and more readily than normal yarn. The polymerized oil, besides 50 affecting the characteristics, such as the shape and type formed, acts as a solvent for the colors, thereby aiding in their dispersion. The yarn treated according to my invention requires less dye than normal yarn to obtain a similar shade.

55 Yarn treated according to my invention is very easily delustered, exhibiting a pronounced loss of lustre when subjected to conditions under

which normal yarn exhibits but a faint or doubtful trace of delustre.

A textile knitted from the yarn processed in accordance with this invention has a very soft handle and does not feel sticky to the hand. The 5 yarn knits with a free stitch and gives a fabric which has a very much smaller number of pin holes, etc., than is obtained with normal yarn under similar conditions.

In accordance with my invention, I propose to 10 add to the spinning solution for the formation of artificial filaments, sheets and the like between 1 and 20% of a polymerized oil such as castor oil and like oils.

15 It was found that many of the oils, such as castor oil, polymerized more readily in the presence of catalyst such as the metals cobalt, cerium or vanadium, or acids such as boric acid or the acids of the third group of the periodic table. There are methods of removing the catalyst from 20 the polymerized oil but this is unnecessary in their use in accordance with my invention. Although certain beneficial results are obtained in using the polymer of a highly purified oil and also in removing the catalyst from the polymerized 25 oil, there are also additional beneficial results obtained by leaving the catalyst in the polymerized oil.

30 By polymerized oil I mean to include also the gels or colloids formed from the oils.

35 By way of illustrating my invention still further but without limiting its scope thereby, I give the following specific examples:

## Example I

35

A spinning charge was prepared by dissolving cellulose acetate in 95/5, acetone /H<sub>2</sub>O, so that a 26% solution of cellulose acetate was obtained. To this solution was added 10% of castor oil polymerized with boric acid as catalyst, the amount of oil being calculated on the weight of the cellulose acetate in the solution, the polymerized oil also containing the catalyst employed in the polymerization thereof. After the usual filtration through filter presses and the like, the charge was dry spun. The spinning stability was an improvement over normal spinning solutions. The yarn appeared normal and bright but took dye more readily and dyed to a darker shade than normal yarn. The yarn has a great 40 advantage over normal yarn in that it takes a dye quicker and more evenly and is easily delustered. The yarn was successfully knitted into a 45 course fabric with 12 feeds.

45

50

55

60

## Example II

Cellulose acetate yarn of 150 denier was spun from a normal spinning solution with a normal lustre. A 50% solution of polymerized castor oil, with the boric acid catalyst remaining therein, 60

in monoethylether of ethylene glycol was applied to the yarn at the spinning cabinet by means of a roller. The treated yarn was aged 5 days and knitted on a 20" diameter 12 feed machine. The 5 fabric was dyed and scoured. The fabric had a soft handle and was free from pin holes and dyed more readily and evenly than normal fabric.

It is found that 5% of the polymerized oil does not gum the filaments together and the yarn finished therewith has quite a softer handle than 10 normal yarn and does not feel sticky to the hand.

*Example III*

Same as Example II except that a 50/50 mixture of polymerized oil with a wax-like body (diglycol stearate) was applied to the yarn. The 15 yarn was finished with 5% of the mixture applied from a 35% solution of butyl acetate at 50° C.

A very much improved fabric having a good 20 knit and a soft handle was formed from the yarn thus treated.

The polymerized or gelled oils may be used in 25 a mixture with wax-like materials and wax-like bodies such as diglycol stearate or any of the ethylene glycol stearates or oleates, any of the glycerol oleates or stearates, triethanolamine oleate or stearate, or glycol or glycerol esters or ethers. Other similar wax-like bodies may be used, such as the palmitates and the substituted 30 glycols and/or glycerols of the fatty acids. These may be used alone or any number of them may be mixed with the polymerized oil and in any percentage, preferably, however, in ratios between 25/75 and 75/25.

The polymerized oils may be incorporated in 35 the spinning solution or in the yarn spun from any solvent compatible therewith such as acetone, butyl acetate, monoethyl ether of ethylene glycol etc. when used with or on cellulose acetate. Both 40 the polymerized oils and mixtures of these with the wax-like bodies may be applied from solvents having an evaporation rate and polarity similar to butyl acetate.

The oils may be polymerized or gelled to any 45 consistency from a liquid through paste to a solid. In the preferred form, as when using castor oil-boric acid, the oil is polymerized to a light straw colored rigid gel which in spite of its rigidity, after 50 breaking or cutting is yet capable of healing back to a single solid piece.

It is to be understood that the foregoing detailed description is given merely by way of illustration and that many variations may be made 55 therein without departing from the spirit of my invention.

Having described my invention, what I desire to secure by Letters Patent is:

1. The process of producing artificial textile material of improved properties comprising adding to the textile material a polymerized but substantially non-oxidized oil.

2. The process of producing artificial yarns and filaments of improved properties comprising incorporating a polymerized but substantially non-oxidized oil in said artificial yarns and filaments.

3. The process of producing artificial yarns and filaments of improved properties comprising adding a polymerized but substantially non-oxidized oil to a spinning solution and forming the 65 filaments therefrom.

4. The process of improving the properties of a textile material which comprises incorporating in the textile material containing organic derivatives of cellulose a polymerized but substantially 70 non-oxidized oil and a wax-like body.

5. The process of improving the properties of yarns or filaments containing cellulose acetate comprising applying thereto 1 to 20% of polymerized but substantially non-oxidized oil.

6. The process of improving the properties of 5 yarns or filaments containing cellulose acetate, comprising applying thereto a polymerized but substantially non-oxidized oil and a wax-like body.

7. The process of improving the properties of 10 artificial material containing a cellulose derivative which comprises treating the material with a swelling agent and a polymerized but substantially non-oxidized oil.

8. The process of improving the properties of 15 artificial materials containing a derivative of cellulose which comprises treating the material with a swelling agent, a polymerized but substantially non-oxidized oil and a wax-like body.

9. The process of improving the properties of 20 artificial textile materials comprising applying thereto a polymerized but substantially non-oxidized oil in a solvent.

10. The process of improving the properties of 25 textile materials comprising adding thereto an oil that has been polymerized in the presence of a catalyst, the catalyst remaining in the polymerized oil.

11. The process of improving the properties of 30 textile materials comprising adding thereto a wax-like body and an oil that has been polymerized in the presence of a catalyst, the catalyst remaining in the polymerized oil.

12. The process of improving the properties of 35 textile materials containing organic derivatives of cellulose comprising adding thereto castor oil that has been polymerized in the presence of a boric acid catalyst, the boric acid catalyst remaining in the polymerized oil.

13. The process of improving the properties of 40 textile materials containing cellulose acetate comprising adding thereto a wax-like body and castor oil that has been polymerized in the presence of a boric acid catalyst, the boric acid catalyst remaining in the polymerized oil. 45

14. Artificial yarns and filaments of improved textile properties containing a polymerized but substantially non-oxidized oil.

15. Artificial yarns and filaments of improved 50 textile properties containing a polymerized castor oil and a wax-like body.

16. Yarns and filaments containing derivatives of cellulose and polymerized but substantially non-oxidized oil. 55

17. Yarns and filaments containing cellulose acetate and polymerized castor oil.

18. The process of producing artificial textile material of improved properties comprising adding to the textile material polymerized castor oil. 60

19. The process of producing artificial yarns and filaments of improved properties comprising incorporating polymerized castor oil in said artificial yarns and filaments.

20. The process of improving the properties of 65 yarns or filaments containing cellulose acetate comprising applying thereto 1 to 20% of polymerized castor oil.

21. The process of improving the properties of 70 textile materials comprising adding thereto castor oil that has been polymerized, in the presence of a catalyst, the catalyst remaining in the polymerized castor oil.

CERTIFICATE OF CORRECTION.

Patent No. 2,041,728.

GEORGE SCHNEIDER.

May 26, 1936.

It is hereby certified that error appears in the printed specification of the above numbered patent requiring correction as follows: Page 1, first column, line 54, before "formed" insert the words of the filaments; and that the said Letters Patent should be read with this correction therein that the same may conform to the record of the case in the Patent Office.

Signed and sealed this 21st day of July, A. D. 1936.

Henry Van Arsdale

(Seal)

Acting Commissioner of Patents.